

Nov. 28, 1933.

H. D. RICE

1,936,994

RUBBER INSULATED ELECTRICAL CONDUCTOR

Filed Aug. 5, 1931



Fig. 1.



Fig. 4.



Fig. 2.



Fig. 5.



Fig. 3.



Fig. 6.

INVENTOR  
HAROLD D. RICE  
BY  
*Walter N. Piper*  
ATTORNEY

## UNITED STATES PATENT OFFICE

1,936,994

## RUBBER INSULATED ELECTRICAL CONDUCTOR

Harold D. Rice, Bristol, R. I., assignor to National India Rubber Company, Bristol, R. I., a corporation of Rhode Island

Application August 5, 1931. Serial No. 555,209

9 Claims. (Cl. 173—264)

This invention relates to rubber insulated electrical conductors and methods of manufacturing the same.

This is a continuation, as to all common subject matter therein, of application No. 388,036 filed August 23, 1929.

Heretofore it has been the practice to apply rubber insulation to electrical conductors by either extruding the rubber onto the conductor, or by forming the rubber in sheet form, cutting the sheets into strips, and wrapping the strips about the conductor and vulcanizing. The conductor is usually protected from direct contact with the rubber by covering with tin, a cotton serving, paper, or a combination of these, prior to the application of the rubber. After vulcanization, the conductor is finished by methods well known in the art, by braiding single, by laying up in parallel, or twisting, with or without a braid, and finally covering if desired with silk, rayon, or cotton braids, or the like, or reinsulating with a rubber compound.

It is the object of this invention to provide a rubber insulation for conductors which is of a grainless texture, is unmilled, and which is tough, flexible, durable and has a high resistance to abrasion.

It is also the object of this invention to apply a suitable rubber insulation to a conductor directly from latex or other aqueous dispersions of rubber.

It is the further object of this invention to provide an insulation for an electrical conductor from an aqueous dispersion of rubber that has high electrical insulating properties especially when wet.

It is also the object of the invention to provide improved constructions of various types of electrical conductors.

Other objects and advantages of the present invention will appear from the following description.

In the drawing is shown various embodiments of the invention; in which

Figure 1 illustrates a solid conductor, insulated, and braided single;

Fig. 2 illustrates a stranded conductor, insulated, layed up in parallel, and braided double;

Fig. 3 illustrates another construction of stranded conductor, insulated, layed up in parallel, and braided double;

Fig. 4 illustrates an insulated solid conductor such as code wire;

Fig. 5 illustrates a stranded conductor, insu-

lated, twisted double, and with an overall re-insulation of rubber; and

Fig. 6 illustrates a stranded conductor, insulated, twisted double with a filler, and with an overall re-insulation of rubber.

The conductor to be insulated is brought to size on wire drawing machinery if a solid conductor, or made in stranded form if of a flexible construction, in a manner well known in the art. The conductor may be tinned, paper wrapped, or provided with a serving of cotton or other fibrous material prior to the application of the rubber insulation thereon. Such a covering, as is well known, protects the wire from the action of free sulphur contained in the rubber composition which otherwise would migrate into contact with the copper of the wire to produce an undesirable reaction.

The conductor preferably tinned, or served with cotton or other fibrous material, or both tinned and served with fibrous material may then be conducted into and through a bath of an aqueous dispersion of rubber which preferably takes the form of latex which has been purified and compounded with vulcanizing ingredients

and if desired also filler ingredients. As the conductor emerges from the coating bath, it is preferably passed through a drying chamber to coagulate the rubber, or the solid constituents of the adhering dispersion may be deposited in any other suitable manner as by acid coagulation,

for example. The latex used preferably contains vulcanizing ingredients and an accelerator which may be set off during passage of the conductor through the drying chamber, where

sufficient heat may be employed to produce a vulcanization of the rubber coating. Of course, if desired, only enough heat to dry the rubber need be employed and the vulcanization may be completed by a subsequent heating operation.

The rubber in the dispersion may, if desired, be in vulcanized condition, and in such case, a lower temperature and smaller drying chamber may be used than when vulcanization is also effected.

The dipping and drying or dipping and coagulating operations may be repeated until a sufficient thickness of rubber has been formed on the wire to provide a layer having the desired electrical insulation properties.

In Figures 1 and 2 are illustrated examples of conductors made according to the present invention. Figure 1 illustrates a conductor in which

1 represents a solid core, 2 a cotton serving thereover, 3 a layer of rubber deposited from an aqueous dispersion of rubber over the serving, and 4

60

70

75

80

85

90

95

100

105

110

a final braid over the insulation on the single conductor. Figure 2 illustrates a pair of parallel stranded conductors such as may be used for lamp cord, in which 5 represents the stranded cores, 6 a cotton serving over the cores, 7 a layer of rubber deposited from an aqueous dispersion of rubber over the serving, and 8 an overall braiding over the two conductors made of fibrous material, such as cotton or rayon, or the like. Conductors insulated with rubber from an aqueous dispersion of rubber may be finished in a variety of ways. For single conductors, they may be finished with a braid as shown in Figure 1. For multiple conductors, a plurality of the 15 rubber insulated wires, either with or without a braid over each wire, may be finished by braiding overall, as shown in Figure 2.

For still heavier insulations, and where even a greater toughness, durability, and resistance to abrasion is desired, the single conductors insulated and braided may again be passed through a rubber dispersion and dried or otherwise coagulated. As before this may be repeated any number of times, depending upon the thickness 25 of the layer of insulation desired. This dipping in the dispersion again after the wire has been coated with a film of rubber and a braid has been provided over the rubber, impregnates the braid and also sufficient dispersion passes through 30 the braid so that on subsequent drying, and vulcanization, the new film of rubber over the braid is bonded through the braid to the inner rubber film. Such a novel construction of a rubber film over the braid which also provides a bond with 35 the inner rubber film through the braid, provides an exceptional insulation. Conductors formed in this manner may be finished in the same manner as the conductors with one layer of rubber insulation above, either by braiding 40 for single conductor, or braiding overall a plurality of conductors with or without a braid over the single wires, or by reinsulating overall with a rubber compound. Figure 3 illustrates as one form of such construction a pair of parallel 45 stranded conductors such as may be used for lamp cord, in which 9 represents the stranded cores, 10 a cotton serving over the cores, 11 a layer of rubber deposited from an aqueous dispersion of rubber over the serving, 12 a braid 50 of fibrous material, for example, cotton over said film. Over this braid 12 another film 13 of rubber bonded to the first film 11 through the braid 12, is deposited from an aqueous dispersion of rubber, and 14 represents an overall braiding 55 over the two conductors made of a fibrous material, such as cotton, rayon, or the like.

Figure 4 illustrates a solid conductor such as code wire in which 15 represents the usual tinned solid conductor and 16 a layer of rubber deposited 60 from an aqueous dispersion of rubber over the core.

Figures 5 and 6 illustrate conductors which are twisted in pairs and have an overall reinsurance of rubber deposited from an aqueous dispersion of rubber. Figure 5 illustrates a pair of twisted stranded conductors in which 17 represents the stranded cores, 18 a cotton serving over the cores, 19 a layer of rubber deposited from an aqueous dispersion of rubber over the serving and 20 an overall reinsurance over the twisted conductors 65 of rubber deposited from an aqueous dispersion of rubber. Figure 6 illustrates a pair of twisted stranded conductors in which 21 represents the stranded cores, 22 a cotton serving over the cores, 23 a layer of rubber deposited from an aqueous

dispersion of rubber over the serving, 24 a pair of fillers made of twisted cotton threads, 25 a coarse net like overall braid of cotton and 26 an overall reinsurance over the twisted conductors and fillers of rubber deposited from an aqueous dispersion of rubber. Of course, the reinsurance 80 20 and 26 may, if desired, be tubed, if desired from a solid rubber composition in the usual manner.

Insulation deposited from normal latex or other aqueous dispersions of rubber which contain a high percentage of water soluble non-rubber ingredients have inferior electrical insulating properties, especially when moist. I have found that a purification of the latex such as a reduction of the amount of non-rubber ingredients in the latex composition by purification processes such as disclosed and claimed in the Hopkinson and Gibbons Patent Reissue 16,874, by dialysis or electrodialysis, or by creaming processes such as 90 with the aid of creaming agents and/or centrifuging provides a latex from which insulation may be made which has high electrical insulating properties, even when wet. As an example, I may use a latex twice creamed with pectin or alginates 95 or Irish moss or other suitable creaming agents, forming a creamed latex of 50-60% solids. Whereas a normal latex contains about 11 or 12% of solid non-rubber constituents which includes soaps, resins, proteins, salts quebrachitol 100 and smaller amounts of other materials, and concentrated latex even a greater percentage, a once creamed latex contains approximately but 4-5% of solid non-rubber constituents and a twice creamed latex contains from 2 1/2-3% non-rubber 105 constituents, and if the creaming process is continued the amount of non-rubber constituents may be even further decreased. On the other hand, the best known types of crude rubber have anywhere from 7 to 8% solid non-rubber constituents. In order to form the best electrical insulation from an aqueous dispersion of rubber, the amount of solid non-rubber constituents should be kept as low as possible. The removal of practically all of the water soluble constituents contained in the latex, as by creaming, renders the rubber dispersion most satisfactory for use in forming rubber insulation.

The following examples of insulation compositions are merely included as illustrations and 125 are not intended to be construed in any way as limitations of the invention:

#### Example 1

|                                     | Parts |
|-------------------------------------|-------|
| Rubber as creamed latex             | 100   |
| Zinc oxide                          | 4     |
| Sulphur                             | 3     |
| Whiting                             | 10    |
| Zinc dimethyl amino dithiocarbamate | 1/2   |
| Ammonium stearate                   | 1     |
| Sodium undecylenate (25% solution)  | 2     |

#### Example 2

|                                     | Parts |
|-------------------------------------|-------|
| Rubber as creamed latex             | 100   |
| Zinc oxide                          | 4     |
| Sulphur                             | 3     |
| Whiting                             | 25    |
| Asphalt                             | 25    |
| Zinc dimethyl amino dithiocarbamate | 1/2   |
| Ammonium stearate                   | 1     |

## Example 3

|                                     | Parts |
|-------------------------------------|-------|
| Rubber as creamed latex             | 100   |
| Zinc oxide                          | 1     |
| 5 Sulphur                           | 3     |
| Zinc dimethyl amino dithiocarbamate | 1/2   |
| Ammonium stearate                   | 1     |

Examples 1 and 2 illustrate latices creamed once or more times as desired, containing vulcanizing ingredients and also filler materials. Example 3 illustrates a latex, creamed once or more times as desired, containing vulcanizing ingredients and no compounds other than are necessary for vulcanization purposes. The zinc 15 dimethyl amino dithiocarbamate is an accelerator of vulcanization. The ammonium stearate acts as a stabilizer of the dispersion and increases the penetrating power of the rubber dispersion and thus enables it better to wet the materials such 20 as the cotton service etc. with which it comes in contact. The sodium undecylenate in Example 1 is a stabilizer. The various ingredients may be added dry, in solution, or in suspension in a manner well known in the art. The asphalt in 25 Example 2 is preferably added in the form of an emulsion. The above formulae may be cut with water to any desired solids content. I have found a latex composition compounded to about 40% solids content very satisfactory to apply. 30 Other accelerators and compounding ingredients may be used, if desired. The proportions and nature of the compounding ingredients may obviously be varied to suit the purposes to which the conductor is to be put as will be evident to 35 one skilled in the art. The latices, as described above, may be purified in other ways than by creaming, if desired.

While the invention has been described more or less in detail, it is not intended thereby to so limit the invention inasmuch as the examples herein set forth are merely illustrative thereof and various modifications may be made without departing from the invention, the scope of which is indicated in the following claims.

45 Having thus described my invention, what I claim and desire to protect by Letters Patent is:  
 1. An electrical conductor comprising a core of conducting material and an insulation thereon of vulcanized and grainless unmilled rubber composition containing not more than 5% of natural non-rubber constituents.

2. An electrical conductor comprising a core of conducting material and an insulation thereon of vulcanized and grainless unmilled rubber composition substantially free from water-soluble constituents.

3. An electrical conductor comprising a core of conducting material and an insulation thereon of vulcanized and grainless unmilled rubber composition substantially free from water-soluble constituents and containing not more than 3% natural non-rubber constituents.

4. An electrical conductor comprising a core of conducting material and an insulation thereon of vulcanized and grainless unmilled rubber composition containing not more than 3% natural non-rubber constituents based on the rubber content.

5. An electrical conductor comprising a core of conducting material and an insulation thereon of vulcanized and grainless rubber composition deposited directly from a creamed rubber latex.

6. An electrical conductor comprising a core of conducting material and an insulation thereon of vulcanized and grainless rubber composition deposited directly from a rubber latex from which has been removed the major proportion of natural non-rubber constituents.

7. An electrical conductor comprising a core of conducting material and an insulation thereon of vulcanized and grainless rubber composition deposited directly from rubber latex, said latex containing not more than 5% natural non-rubber constituents on a dry rubber basis.

8. An electrical conductor comprising a core of conducting material and an insulation thereon of vulcanized and grainless rubber composition deposited directly from rubber latex, said latex being substantially free from natural water-soluble constituents.

9. An electrical conductor comprising a core of conducting material and an insulation thereon of vulcanized and grainless rubber composition deposited directly from rubber latex, said latex containing not more than 3% natural non-rubber constituents on a dry rubber basis and being substantially free from natural water-soluble constituents.

HAROLD D. RICE. 125

55

130

60

135

65

140

70

145

75

150